

# UNITED STATES PATENT OFFICE.

RICHARD H. PATCH, OF PHILADELPHIA, AND RADCLYFFE FURNESS, OF JENKINTOWN, PENNSYLVANIA, ASSIGNEES TO THE MIDVALE STEEL COMPANY, OF PHILADELPHIA, PENNSYLVANIA, A CORPORATION OF PENNSYLVANIA.

## TOOL-STEEL ALLOY.

1,206,902.

Specification of Letters Patent.

Patented Dec. 5, 1916.

No Drawing.

Application filed September 16, 1915. Serial No. 50,960.

*To all whom it may concern:*

Be it known that we, RICHARD H. PATCH and RADCLYFFE FURNESS, citizens of the United States, residing at, respectively, 5 Philadelphia, county of Philadelphia, State of Pennsylvania, and Jenkintown, county of Montgomery, State of Pennsylvania, have invented a new and useful Improvement in Tool-Steel Alloys, of which the following is a full, clear, and exact description.

Our invention relates to the production of non-deforming tool steel particularly adapted for dies, taps, reamers, and cutting 15 tools for lathes and planers.

The invention comprises an alloy of steel and chromium combined in certain proportions with carbon.

Following is a typical composition, and 20 one which careful experiment has shown to give an excellent result: Carbon 1.35%, chromium 19.50%, iron 79.00%. The alloy should contain about 1 to 1.50 per cent. of carbon, although, for special uses, this may 25 be raised to 2 per cent. carbon. The chromium should be kept within the range between 15 and 20 per cent.

In the manufacture of tool steel, it is not

new to employ small quantities of chromium, but, hitherto, at least, we believe that 30 it has only been proposed to use chromium between 12 and 16 per cent., with carbon above 2 per cent. The advantage of a tool steel containing the relative proportions of carbon and chromium specified over other 35 chrome steel compositions is an immense increase in the life of the tool and the capacity to cut at substantially higher speeds.

Having now fully described our invention, what we claim and desire to protect 40 by Letters Patent is:

1. A tool steel containing between 15 and 20 per cent. of chromium and between 1 and 2 per cent. of carbon.

2. A tool steel containing the following 45 ingredients in approximately the proportions specified: steel about 79 per cent.; chromium about 19.5 per cent. and carbon about 1.35 per cent.

In testimony of which invention, we have 50 hereunto set our hands at Philadelphia, on this 14th day of September, 1915.

RICHARD H. PATCH.  
RADCLYFFE FURNESS.

Witness:

JAMES J. RAHILLY.